

[54] SILVER HALIDE PHOTOGRAPHIC MATERIAL CONTAINING A SENSITIZING AND STABILIZING COMBINATION OF A POLYALKYLENE OXIDE, A TETRAZAINDENE AND A RESORCINOL DERIVATIVE

[75] Inventors: Teiji Habu; Tomio Nakajima; Eiichi Sakamoto; Kenzi Kadokura; Kyusaku Yoshida; Katsutoshi Machida, all of Hino, Japan

[73] Assignee: Konishiroku Photo Industry Co., Ltd., Tokyo, Japan

[22] Filed: May 8, 1974

[21] Appl. No.: 467,957

[30] Foreign Application Priority Data

May 12, 1973 Japan..... 48-52094

[52] U.S. Cl..... 96/76 R; 96/107; 96/109

[51] Int. Cl.<sup>2</sup> ..... G03C 1/28; G03C 1/34

[58] Field of Search..... 96/107, 109, 95, 76 R

[56] References Cited

UNITED STATES PATENTS

|           |        |                     |        |
|-----------|--------|---------------------|--------|
| 2,418,613 | 4/1947 | Allen et al.....    | 96/109 |
| 2,716,062 | 8/1955 | Carroll et al.....  | 96/109 |
| 3,236,652 | 2/1966 | Kennard et al ..... | 96/109 |
| 3,457,079 | 7/1969 | Koda et al .....    | 96/109 |
| 3,563,754 | 2/1971 | Jones et al.....    | 96/109 |
| 3,671,258 | 6/1972 | Taber.....          | 96/109 |

Primary Examiner—Won H. Louie, Jr.  
Attorney, Agent, or Firm—Bierman & Bierman

[57] ABSTRACT

This invention relates to a light-sensitive silver halide photographic material having a photographic layer incorporated with a polyalkylene oxide type compound, a tetrazaindene type compound and a resorcinol type compound.

4 Claims, No Drawings

**SILVER HALIDE PHOTOGRAPHIC MATERIAL  
CONTAINING A SENSITIZING AND STABILIZING  
COMBINATION OF A POLYALKYLENE OXIDE, A  
TETRAZAINDENE AND A RESORCINOL  
DERIVATIVE**

Recently, light-sensitive silver halide photographic materials are required to have properties satisfying increasingly complex and diverse requirements. Particularly, high speed to ultra-high speed silver halide photographic materials having stable photographic properties are demanded, and, in the radiography, X-ray photographic materials high in speed and free from fog are demanded so as to obtain more informations with smaller doses of X-rays in order that the human body is less exposed to radiation.

It has heretofore been said that for increase in speed of a light-sensitive silver halide photographic material, it is quite effective to incorporate a polyalkylene oxide type compound into the photographic material, as disclosed in, for example, "The Theory of the Photographic Process", Third Edition, pages 369-370 (1967). However, the amount of polyalkylene oxide type compound used in such case is restricted, and if the amount thereof exceeds a definite limit, the photographic material is greatly increased in fog. Furthermore, when the photographic material is subjected, during its preparation, to quick drying under low humidity conditions, or subjected to development under severe conditions at elevated temperatures, the increase of fog is further promoted to cause such fatal disadvantage that the photographic material is greatly deteriorated in photographic properties.

In order to prevent the said high speed silver halide photographic material from formation of fog to stabilize the photographic properties thereof, there have been made attempts to use such tetrazaindene type compounds as disclosed in, for example, Japanese Patent Publication No. 9,432/57 and U.S. Pat. No. 2,716,062. However, the said tetrazaindene compounds are extremely weak in action of preventing the formation of fog and the degradation of photographic properties in the case where the photographic material is subjected to such severe conditions required in recent years that it is prepared through low humidity quick drying steps, stored under high temperature high humidity conditions, or processed under high temperature quick development conditions. Thus, the tetrazaindene type compounds cannot display practical effects. To cope with this, there have been desired proper antifoggants necessary to make the polyalkylene oxide type compound effectively display its action as a sensitizer. However, the actual state is such that no satisfactory antifoggants have been discovered yet.

An object of the present invention is to provide a light-sensitive silver halide photographic material sensitized with a polyalkylene oxide type compound which is high in speed and free from fog and thus is stable in photographic properties.

Another object of the invention is to provide a light-sensitive silver halide photographic material which is free from increase in fog and stable in photographic properties even when subjected to such severe conditions as in the case where it is prepared through low humidity quick drying treatment at the time of coating and drying of silver halide emulsion, stored in a high temperature high humidity atmosphere, or processed under high temperature quick development conditions.

The above-mentioned objects can be accomplished by incorporating, into a light-sensitive silver halide photographic material sensitized with a polyalkylene oxide type compound, at least one compound selected from tetrazaindene type compounds, and at least one compound selected from resorcinol type compounds (hereinafter referred to as "compound A") having the following general formulas I and II:

General formula I:



General formula II:



wherein R<sub>1</sub>s, same or different, are a hydrogen atom, a halogen atom, a hydroxyl group, an alkyl group which may have a substituent, an aralkyl group which may have a substituent, an alkoxy group which may have a substituent, an acyl group which may have a substituent, a carboxymethyl group which may have a substituent, or a group —COOM or —SO<sub>3</sub>M (where M is a hydrogen atom, an alkali metal atom or an ammonium group); R<sub>2</sub> and R<sub>3</sub> are individually a group —COOM or —SO<sub>3</sub>M; and n<sub>1</sub> and n<sub>2</sub> are individually an integer of 1 to 3.

That is, when the said light-sensitive silver halide photographic material sensitized with a polyalkylene oxide type compound is incorporated with a tetrazaindene type compound and a compound A, the sensitizing action possessed by the polyalkylene oxide type compound is effectively displayed to make it possible to obtain a photographic material which is high in speed and free from fog and can maintain stable photographic properties even under such severe conditions as mentioned previously.

The polyalkylene oxide type compound used as a sensitizer for the photographic material according to the present invention includes various compounds such as, for example, polyalkylene glycols, addition polymerization products of alkylene oxides with hexitol ring dehydration compounds, and addition polymerization products of phenol-formalin resins with alkylene oxides. These polyalkylene oxide type compounds should have a molecular weight of at least 300, preferably from 500 to 8,000. Typical examples of these compounds are as follows:

- (P-1) Addition polymerization product of 1 mole of p-t-butylphenol with about 27 moles of ethylene oxide.
- (P-2) Addition polymerization product of 1 mole of nonylphenol-formalin resin with 10 moles of ethylene oxide.
- (P-3) Condensation product of 1 mole of lauryl alcohol with about 20 moles of ethylene oxide.
- (P-4) Polyethylene glycol.
- (P-5) Condensation product of 1 mole of phenol with about 20 moles of ethylene oxide.

(P-6) Addition polymerization product of 1 mole of n-butyl mercaptan with 10 moles of propylene oxide and 20 moles of ethylene oxide.

(P-7) Addition polymerization product of 1 mole of octylphenol-formalin resin with 15 moles of ethylene oxide.

(P-8) Addition polymerization product of 1 mole of p-cresol-formalin resin with 8 moles of ethylene oxide.

(P-9) Addition polymerization product of 1 mole of p-thiocresol with 30 moles of ethylene oxide.

The tetrazaindene type compound used in the present invention includes compounds of various structures. Particularly effective are compounds of the following general formula III:



wherein  $\text{R}_1$  is a hydrogen atom, a carboxyl group, an esterified carboxyl group, a mercapto group, an alkyl group which may have a substituent, an aryl group which may have a substituent, a heterocyclic group which may have a substituent, an alkylthio group which may have a substituent, an aralkylthio group which may have a substituent, or an alicyclic group which may have a substituent;  $\text{R}_2$  is a hydrogen atom, a halogen atom, a carboxyl group, an esterified carboxyl group, an amino group which may have a substituent, an aryl group which may have a substituent, an aralkyl group which may have a substituent, an alicyclic group which may have a substituent, a heterocyclic group which may have a substituent, or a thiuronium group which may have a substituent; and  $\text{R}_3$  is a hydrogen atom, a hydroxyl group, a carboxyl group, an esterified carboxyl group, an amino group which may have a substituent, an alkyl group which may have a substituent, an alicyclic group which may have a substituent, or a heterocyclic group which may have a substituent.  $\text{R}_2$  and  $\text{R}_3$  may form, in combination, a carbocyclic ring or a heterocyclic ring.

Typical examples of the tetrazaindene type compound used in the present invention are as follows:

(T-1)



(T-2)



(T-3)



4



15

(T-5)



25

(T-6)



30

(T-7)



40

(T-8)



50

60

(T-9)



65

5

(T-10)



5

6

(T-17)



10

(T-11)



15

(T-18)



20

(T-12)



25

(T-19)



30

(T-13)



(T-20)



40

(T-14)



45

(T-21)



50

(T-15)



(T-22)



60

(T-16)



65

(T-23)



7

(T-24)



(7)



8

(8)



(T-25)



(9)



15

(10)

(10)



(T-26)



20

(11)



25

(12)



25

(13)



(14)



15

(15)



(16)



40

(1)



(2)



(17)



(18)



(3)



(4)



50

(19)



(20)



(5)



(6)



60

(21)



(22)



65

The above-mentioned tetrazaindene type compounds 30 can be easily synthesized according to the processes described in, for example, "The Journal of Organic Chemistry", Vol. 24, pages 779-801 (1959) and Vol. 25, pages 861-866 (1960), Japanese Patent Publication No. 9,432/57, and U.S. Pat. Nos. 2,716,062, 35 2,835,581 and 2,566,659.

The compound A used in the present invention includes such compounds as mentioned below.

Typical examples of compounds of the aforesaid general formula I are as follows:



Typical examples of compounds of the aforesaid general formula II are as follows:



The above-mentioned compounds A can be easily synthesized according to the processes described in, for example, "Gazzetta Chimica Italiana", Vol. 57, pages 793-802 (1927), "Chemical Abstracts", Vol. 41, page 5495 (1947), "Helvetica Chemica Acta", Vol. 43, page 644 (1960), "Beilsteins Handbuch der Organischen Chemie", Vol. 6, page 987, and Vol. 11, page 304.

The said polyalkylene oxide type compound, tetraazaindene type compound and compound A are preferably made present in the silver halide emulsion layer of a light-sensitive silver halide photographic material, but may be made present in any of protective layer, sub layer or inter layer adjacent to said silver halide emulsion layer. The compounds may be made present either in combination in one layer or independently in separate adjacent layers. At the time of incorporation into a photographic material, the compounds may be brought into the form of a solution or solutions in water or an organic solvent compatible with water such as lower alcohol or ketone, or in a mixed solvent comprising water and organic solvent, and may be added either simultaneously or separately. For example, the polyalkylene oxide type compound as a sensitizer, the tetraazaindene type compound and the compound A may be added in this order.

The time of addition of these compounds to a silver halide emulsion, for example, may be an optional stage during preparation of the emulsion, but is preferably the stage immediately before completion of the second ripening.

The amounts of the compounds to be added to a silver halide emulsion vary depending on the kinds of the compounds and of the silver halide emulsion. Ordinarily, however, the amount of the polyalkylene oxide type compound is preferably in the range from 0.01 to 5 g., and the amount of each of the tetraazaindene type compounds and the compound A is in the range from 0.1 to 50 g., more preferably from 0.5 to 50 g., per mole of the silver halide. The proportion of the compound A is preferably in the range from 0.1 to 10 parts by weight per part by weight of the tetraazaindene type compound.

Silver halide emulsions usable in the light-sensitive silver halide photographic materials of the present invention are black-and-white photographic emulsions, X-ray photographic emulsions, lith-type emulsions, incorporated type and Fischer type color photographic emulsions, and black-and-white and color photographic emulsions for diffusion transfer, and may contain various silver halides such as silver bromide, silver iodobromide, silver chlorobromide and silver chloroiodobromide. Further, the silver halide emulsions may have been sensitized with noble metal sensitizers, chemical sensitizers such as sulfur or reduction sensitizers, or color sensitizers, and may have been incorporated with various photographic additives used hitherto.

The thus prepared light-sensitive silver halide photographic material of the present invention is not only high in speed, free from fog and excellent in gradation, but also have photographic properties capable of withstanding such severe conditions as in the cases where it is prepared through low humidity quick drying treatment at the time of coating and drying of silver halide emulsion, stored under high temperature high humidity conditions, and processed under high temperature quick development conditions.

The present invention is illustrated in detail below with reference to examples, but the examples do not limit the scope of the invention.

#### EXAMPLE 1

Immediately before completion of second ripening, a high speed negative silver iodobromide emulsion containing 1.5 mole% of silver iodide was incorporated with 0.2 g., per mole of the silver halide, of the compound (P-1) as a polyalkylene oxide type sensitizer, in the form of an aqueous solution, and then with 0.3 g., per mole of the silver halide, of the compound (T-1). After completion of second ripening, the emulsion was equally divided into 9 portions. One of the thus formed 9 emulsions was taken up, incorporated with a coating aid and a hardener, coated on a cellulose triacetate film base to dry thickness of 10  $\mu$ , and then dried to prepare a control sample (Sample No. 1). Each of the remaining 8 emulsions was additionally incorporated with 1.0 g. or 3.0 g., per mole of the silver halide, of the compound A shown in Table 1, and then treated in the same manner as in the case of the control sample to prepare 8 kinds of samples (Sample Nos. 2, 3, 4, 5, 6, 7, 8 and 9).

These samples and the control sample were individually exposed, according to the method regulated in JIS

to white light by use of Sensitometer, Model KS-1 (manufactured by Konishiroku Photo Industry Co., Ltd.), and then subjected to high temperature quick development at 40°C. for 30 seconds in a continuous roller-conveying type automatic developing machine, in which development, fixing, water-washing and drying could be effected consistently, by use of a developer of the following composition:

|                               |           |
|-------------------------------|-----------|
| Anhydrous sodium sulfite      | 70 g.     |
| Hydroquinone                  | 10 g.     |
| Anhydrous boric acid          | 1 g.      |
| Sodium carbonate, monohydrate | 20 g.     |
| 1-Phenyl-3-pyrazolidone       | 0.35 g.   |
| Sodium hydroxide              | 5 g.      |
| 5-Methylbenzotriazole         | 0.05 g.   |
| Potassium bromide             | 5 g.      |
| Glutaraldehyde bisulfite      | 15 g.     |
| Glacial acetic acid           | 8 g.      |
| Water to make                 | One liter |

The thus processed samples and control sample were subjected to sensitometry to measure the photographic properties thereof. The results obtained were as set forth in Table 1. In Table 1, the speed is a relative value calculated by assuming as 100 the speed of the control sample (the same shall apply hereinafter).

Table 1

| Sample No. | Kind and amount of compound A (g/mole silver halide) | Photographic properties | Speed | Fog  | Gamma |
|------------|------------------------------------------------------|-------------------------|-------|------|-------|
| 1          | None                                                 |                         | 100   | 0.23 | 1.1   |
| 2          | Compound (1)                                         |                         | 120   | 0.15 | 1.2   |
| 3          | Compound                                             |                         | 130   | 0.10 | 1.2   |
| 4          | Compound (3)                                         |                         | 125   | 0.12 | 1.1   |
| 5          | Compound                                             |                         | 115   | 0.09 | 1.15  |
| 6          | Compound (4)                                         |                         | 105   | 0.15 | 1.15  |
| 7          | Compound                                             |                         | 110   | 0.10 | 1.20  |
| 8          | Compound (29)                                        |                         | 120   | 0.10 | 1.15  |
| 9          | Compound                                             |                         | 130   | 0.09 | 1.20  |

As is clear from Table 1, it is understood that even when subjected to high temperature quick development, a light-sensitive silver halide photographic material sensitized with a polyalkylene oxide type compound can show fog-free and high speed photographic properties, so far as the photographic material has been further incorporated with the combination of a tetrazaindene type compound and a compound A.

### EXAMPLE 2

A silver iodobromide X-ray photographic emulsion containing 2 mole% of silver iodide was subjected to second ripening by addition of a gold sensitizer, and then incorporated with a hardener, a coating aid and the compound (T-2). Subsequently, the emulsion was equally divided into 9 portions. One of the thus formed 55 emulsions was taken up, and coated on a polyethylene terephthalate film base to a dry thickness of 10  $\mu$  to form a silver halide emulsion layer. On the thus formed layer, a 3% aqueous gelatin solution incorporated with 0.1 g., per gram of gelatin, of the compound (P-2) as a polyalkylene oxide type sensitizer was coated to form a protective layer. The film having the thus protected silver halide emulsion layer was quickly dried in 60 10 minutes in an atmosphere kept at 35°C. and a relative humidity of 40% to prepare a control sample (Sample

No. 10). Each of the remaining 8 emulsions was incorporated with 1.5 g. or 3.0 g., per mole of the silver halide, of the compound A shown in Table 2, and then treated in the same manner as in the case of the control sample to prepare 8 kinds of samples (Sample Nos. 11, 12, 13, 14, 15, 16, 17 and 18).

The thus prepared samples and control sample were individually exposed for 0.5 second to X-rays at a voltage of 60 KV and a peak current of 200 mA, through a fluorescent medical X-ray screen having a medium sensitivity (KYOKKO FS, having a fluorescence spectrum maximum of 4250 Å; produced by Dainihon Paint Co., Ltd.) and through an aluminum optical wedge having a step difference of  $\sqrt{2}$ . Subsequently, the samples and control sample were subjected to the same development and treatment as in Example 1 to measure the photographic properties thereof. The results obtained were as set forth in Table 2.

Table 2

| Sample No. | Kind and amount of compound A (g/mole silver halide) | Photographic properties | Speed | Fog  |
|------------|------------------------------------------------------|-------------------------|-------|------|
| 10         | None                                                 |                         | 100   | 0.31 |
| 11         | Compound (19)                                        |                         | 110   | 0.17 |
| 12         | Compound                                             |                         | 120   | 0.15 |
| 13         | Compound (20)                                        |                         | 105   | 0.20 |
| 14         | Compound                                             |                         | 110   | 0.17 |
| 15         | Compound (23)                                        |                         | 120   | 0.19 |
| 16         | Compound                                             |                         | 135   | 0.12 |
| 17         | Compound (28)                                        |                         | 115   | 0.20 |
| 18         | Compound                                             |                         | 125   | 0.15 |

As is clear from Table 2, it is understood that even when quickly dried under high temperature high humidity conditions, a light-sensitive silver halide X-ray photographic material containing a polyalkylene oxide type compound in the protective layer can give a clear X-ray image high in sensitivity and free from fog, so far as the photographic material has been incorporated with a tetrazaindene type compound and a compound A.

### EXAMPLE 3

Immediately before completion of second ripening, the same silver iodobromide emulsion as in Example 2 was incorporated with 0.2 g., per mole of the silver halide, of the compound (P-3) as a polyalkylene oxide type sensitizer, and then with 0.3 g. per mole of the silver halide, of the compound (T-4). After completion of second ripening, the emulsion was equally divided into 6 portions. One of the thus formed 6 emulsions was taken up, coated on a cellulose triacetate film base, and then dried to prepare a control sample (Sample No. 19). Each of the remaining 5 emulsions was incorporated with a compound A shown in Table 3, and then treated in the same manner as in the case of the control sample to prepare 5 kinds of samples (Sample Nos. 20, 21, 22, 23 and 24).

The thus prepared samples and control sample were subjected to the same development and sensitometry as in Example 1 to measure the photographic properties thereof. The results obtained were as set forth in Table 3.

Table 3

| Sample No. | Kind and amount of compound A (g/mole silver halide) | Photographic properties (storage test) |      |                                   |      |                 |      |
|------------|------------------------------------------------------|----------------------------------------|------|-----------------------------------|------|-----------------|------|
|            |                                                      | Stored for 3 days at 20°C. RH 60%      |      | Stored for 3 days at 50°C. RH 80% |      | Speed Fog Gamma |      |
|            |                                                      | Speed                                  | Fog  | Speed                             | Fog  | Gamma           |      |
| 19         | None                                                 | 100                                    | 0.25 | 1.15                              | 87   | 0.37            | 1.10 |
| 20         | Compound (25)                                        | 2.75                                   | 105  | 0.20                              | 1.18 | 100             | 0.22 |
| 21         | Compound (26)                                        | 2.75                                   | 115  | 0.18                              | 1.20 | 115             | 0.19 |
| 22         | Compound (18)                                        | 3.0                                    | 128  | 0.15                              | 1.19 | 130             | 0.15 |
| 23         | Compound (23)                                        | 3.0                                    | 132  | 0.12                              | 1.21 | 130             | 0.13 |
| 24         | Compound (14)                                        | 2.75                                   | 120  | 0.14                              | 1.20 | 122             | 0.14 |

As is clear from Table 3, it is understood that even when stored for a long period under high temperature 15 high humidity conditions, a high speed silver halide photographic material sensitized with a polyalkylene oxide type compound can maintain high speed and fog-free photographic properties, so far as the photographic material has been further incorporated with a tetrazaindene type compound and a compound A.

## EXAMPLE 4

A silver iodobromide emulsion containing 5 mole% of silver iodide was incorporated with 0.4 g., per mole 25 of the silver halide, of the tetrazaindene compound (T-6). A portion of the silver halide emulsion was taken up, coated on a cellulose triacetate film base, and then dried to prepare a control sample (Sample No. 25). The remaining silver halide emulsion was equally divided into 5 portions. Each of the thus formed 5 emulsions was incorporated with 0.1 g., per mole of the 30 silver halide, of such polyalkylene oxide type compound as shown in Table 4. A portion of each of said 5 emulsions was taken up, coated on a cellulose triacetate film base, and then dried to prepare 5 kinds of control samples (Sample Nos. 26, 29, 32, 35 and 38). Finally, each of the said 5 emulsions was equally divided into 2 portions, and each of the resulting 10 emulsions was incorporated with 3.0 g., per mole of the 35 silver halide, of such compound A as shown in Table 4, and then treated in the same manner as in the case of the control sample to prepare 10 kinds of samples (Sample Nos. 27, 28, 30, 31, 33, 34, 36, 37, 39 and 40).

The thus prepared 6 kinds of control samples and 10 kinds of samples were subjected to the same development and sensitometry as in Example 1 to measure the photographic properties thereof. The results obtained were as set forth in Table 4.

Table 4

| Sample No. | Polyalkylene type compound | Kind and amount of compound A (g/mole silver halide) | Photographic properties |      |
|------------|----------------------------|------------------------------------------------------|-------------------------|------|
|            |                            |                                                      | Speed                   | Fog  |
| 25         | —                          | —                                                    | 100                     | 0.14 |
| 26         | Compound (P-4)             | —                                                    | 115                     | 0.28 |
| 27         | "                          | Compound (24)                                        | 0.3                     | 140  |
| 28         | "                          | "(29)                                                | "                       | 155  |
| 29         | Compound (P-5)             | —                                                    | 110                     | 0.24 |
| 30         | "                          | Compound (24)                                        | "                       | 140  |
| 31         | "                          | "(29)                                                | "                       | 135  |
| 32         | Compound (P-6)             | —                                                    | 120                     | 0.26 |
| 33         | "                          | Compound (24)                                        | "                       | 160  |
| 34         | Compound (P-6)             | Compound (29)                                        | 0.3                     | 170  |
| 35         | Compound (P-7)             | —                                                    | 123                     | 0.27 |
| 36         | "                          | Compound (24)                                        | "                       | 160  |
| 37         | "                          | "(29)                                                | "                       | 150  |
| 38         | Compound (P-8)             | —                                                    | 118                     | 0.24 |
| 39         | "                          | Compound (24)                                        | "                       | 145  |
| 40         | "                          | "(29)                                                | "                       | 160  |

As is clear from Table 4, it is understood that even a light-sensitive silver halide photographic material sensi-

tized with any of such typical polyalkylene oxide type compounds as shown in Table 4 can maintain high speed and fog-free photographic properties, so far as the photographic material has been incorporated with a tetrazaindene type compound and a compound A.

## EXAMPLE 5

A blue-sensitive silver halide color photographic emulsion containing 5 mole% of silver iodide was subjected to second ripening, and then incorporated with, per mole of the silver halide, 0.1 g. of the compound (P-7) as a polyalkylene oxide type sensitizer, 0.3 g. of the compound (T-12), and then 70 g. of 4-dodecylbenzoyl-2'-methoxyacetanilide as a yellow coupler. Subsequently, the emulsion was equally divided into 7 portions. One of the thus formed 7 emulsions was taken up, coated on a cellulose triacetate film base, and then dried to prepare a control sample (Sample No. 41). Each of the remaining 6 emulsions was incorporated with such compound A as shown in Table 5, and then treated in the same manner as in the case of the control sample to prepare samples (Sample Nos. 42, 43, 44, 45, 46 and 47).

The thus prepared samples and control sample were individually developed at 24°C. for 5 minutes by use of a developer of the following composition:

|                                                                      |           |
|----------------------------------------------------------------------|-----------|
| Benzyl alcohol                                                       | 3.8 ml.   |
| Anhydrous sodium sulfite                                             | 2.0 g.    |
| N-Ethyl-N-β-methylsulfonylamidoethyl-3-methyl-4-aminoaniline sulfate | 5.0 g.    |
| Sodium carbonate, monohydrate                                        | 50.0 g.   |
| Sodium bromide                                                       | 1.0 g.    |
| Water to make                                                        | One liter |

Photographic properties of the samples and control samples were as set forth in Table 5.

Table 5

| Sample No. | Kind and amount of compound A (g/mole silver halide) | Speed | Fog  | Photographic properties Gamma |
|------------|------------------------------------------------------|-------|------|-------------------------------|
| 41         | —                                                    | 100   | 0.21 | 0.71                          |
| 42         | Compound (9)                                         | 2.75  | 120  | 0.14 0.77                     |
| 43         | " (9)                                                | 3.25  | 115  | 0.12 0.74                     |
| 44         | " (24)                                               | 2.75  | 135  | 0.12 0.76                     |
| 45         | " (24)                                               | 3.25  | 130  | 0.10 0.77                     |
| 46         | " (23)                                               | 2.75  | 145  | 0.10 0.73                     |
| 47         | " (23)                                               | 3.25  | 150  | 0.11 0.75                     |

As is clear from Table 5, it is understood that a light-sensitive silver halide color photographic material sensitized with a polyalkylene oxide type compound and containing a coupler can also give a brilliant color image high in speed and fog-free, so far as the photographic material has been incorporated with a tetrazaindene type compound and a compound A.

What we claim is:

1. A light-sensitive silver halide photographic material which comprises a light-sensitive silver halide emulsion layer and an adjacent layer thereof, at least one of which contains 0.01 to 5 g, per mole of silver halide, of at least one compound selected from polyalkylene oxide compounds; 0.1 to 50g, per mole of silver halide, of at least one compound selected from tetrazaindene compounds; and 0.1 to 50g, per mole of silver halide, of at least one compound represented by the general formula I or II,



wherein the R<sub>1</sub>'s are individually hydrogen, halogen, alkyl, aralkyl, alkoxy, acyl, carboxymethyl or a group COOM or  $-\text{SO}_3\text{M}$ , M is hydrogen, an alkali metal or ammonium R<sub>2</sub> and R<sub>3</sub> are individually group  $-\text{COOM}$  or  $-\text{SO}_3\text{M}$ ; and n<sub>1</sub> and n<sub>2</sub> are individually 1 to 3.

2. A light-sensitive silver halide photographic material according to claim 1 wherein said tetrazaindene compounds are represented by the following general formula:



wherein R<sub>1</sub> is hydrogen, carboxyl, esterified carboxyl, 45 mercapto, alkyl, aryl, heterocyclic, alkylthio, aralkylthio, or alicyclic; R<sub>2</sub> is hydrogen, halogen, carboxyl, esterified carboxyl, amino, aryl, aralkyl, alicyclic, heterocyclic, or thiuronium; and R<sub>3</sub> is hydrogen, hydroxyl, carboxyl, esterified carboxyl, amino, alkyl, alicyclic, heterocyclic, or R<sub>2</sub> and R<sub>3</sub> can cooperatively 50 form a carbocyclic or hetero ring.

3. A light-sensitive silver halide photographic material according to claim 1 wherein the weight ratio of the amount of the compound represented by the general formula I or II to the amount of the tetrazaindene compound is from 0.1 - 1 to 10 - 1.

4. A light-sensitive silver halide photographic material according to claim 1 wherein the compound of the general formula I or II is selected from the following 60 compounds:





\* \* \* \* \*